

3,684,463  
JEWELRY PRODUCTS  
Franz Koelbl, Salzburg-Parsch, Austria, assignor to  
Schwarzkopf Development Corporation, New York,  
N.Y.  
No Drawing. Filed Nov. 27, 1968, Ser. No. 779,635  
Claims priority, application Austria, Dec. 1, 1967,  
10,854/67  
Int. Cl. B22f 1/00  
U.S. CL. 29—182.8

8 Claims 10

## ABSTRACT OF THE DISCLOSURE

This invention pertains to the manufacture of jewelry and to articles of jewelry having the physical appearance of gold but improved scratch resistance and containing a major amount of a metal selected from the group consisting of tantalum carbide, zirconium nitride, titanium nitride and vanadium nitride and a binder from the group consisting of iron, cobalt, nickel and their alloys.

This invention relates to the jewelry art and, more particularly, to the manufacture of articles of jewelry that are similar in appearance to gold jewelry but at the same time are relatively resistant to scratch and crushing.

The articles of jewelry manufactured in accordance with this invention contain at least 70% by volume and up to 97% by volume of metals selected from the group consisting of tantalum carbide, zirconium nitride, titanium nitride and vanadium nitride. The jewelry articles can contain one of the foregoing metals or it can utilize a mixture of two or more of the aforesaid primary metals, as long as the total concentration of primary metal remains within the aforesaid range.

Preferably, the primary metal will be present in the articles of jewelry in an amount of from about 85 to 90% by volume.

The particular primary metal to be employed in any instance will depend to some extent upon the characteristics desired of the final product. Where it is desired that the article of jewelry approach very closely not only the physical appearance but also the specific gravity of gold, then tantalum carbide is the preferred primary metal. Where a somewhat lesser specific gravity is desired, one of the other primary metals can be employed.

The articles of jewelry should contain, in addition to primary metal, a suitable auxiliary metal. The auxiliary metal must be a metal having a melting point lower than the primary metal, preferably at least about 50° C. less. The auxiliary metal must also be capable of wetting the primary metal employed at the sintering temperature. Iron, cobalt and nickel and alloys of each of them, meeting the foregoing criteria, are satisfactory auxiliary metals.

Nickel is the preferred auxiliary metal either by itself in the form of the commercial grade or pure nickel or in the form of alloys of nickel and chromium. Suitable nickel-chromium alloys will contain from about five to fifty percent by volume of chromium. In such nickel-chromium alloys, copper can also be present in an amount from 1 to 30% by volume. When copper is present in the nickel-chromium alloy, the total volume of chromium and nickel combined should not be greater than the volume of nickel. A preferred auxiliary metal is an alloy containing 80 parts by volume of nickel and 20 parts by volume of chromium. Nickel-molybdenum alloys are also suitable.

The quantity of auxiliary metal is preferably present in an amount of up to 20% by volume in the finished product. For some applications, particularly when used along with titanium nitride, up to 30% by volume of auxiliary metals can be added. Most preferably, the auxiliary metal should be present in an amount of at least 10%.

The combinations of auxiliary and primary metals can be varied so as to achieve particularly desirable properties. For example, a material can be achieved which will be completely non-magnetic. Such a material would be useful for watch cases or the like. Using other combinations of primary and auxiliary metals, the material achieved will be only weakly ferromagnetic, having a saturation value of  $4\pi\sigma$  lower than 20 gauss. In all instances, the product retains the characteristic color and outward physical appearance of gold.

The gold colored articles made by means of this invention are particularly useful when formed into items of jewelry such as, for example, watch cases, watch bracelets and bands, rings, bracelets, charms and pins of all types. Utility is not, of course, limited to jewelry but can be used for other ornamental or utilitarian purposes where the cold coloration is necessary or desirable along with the strength and scratch resistance produced by this invention.

The articles of this invention are prepared by conventional powder metallurgical techniques from powdered starting materials. The primary metal or metals along with any auxiliary metals are obtained and mixed in powdered form, pressed into the desired form, and thereafter sintered. Conventional lubricants can also be added to the mixture to facilitate pressing.

The particle size of the powder is as in conventional powder metallurgical processes. Sintering will take place at the desired sintering temperature for the composition used, the temperature being within the range of 1200 to 2200° C. and for a time to achieve complete sintering. Sintering preferably takes place in a protective atmosphere, i.e., an atmosphere that is non-reactive with the metallic components present. Thus, for example, sintering can take place after evacuation of air or it can take place in an atmosphere of an inert gas such as argon.

Alternatively, the powder mixture can be hot pressed into the desired shape in a mold or other pressure device heated to the sintering temperature with a pressure of from about 50 to 350 kg. per cm.<sup>2</sup> and a time of at least about 2 to 10 minutes.

Where it is desired to machine an item such as a watch case, the powder mixture can be compressed to bring the particles together into the proper shape, pre-sintered only very briefly and then finally sintered at some later date. Because of the hardness of the product, machining may require the use of diamond tools.

After sintering, whether in an oven or through hot pressing, has been completed, the final article is then finished by grinding and polishing to bring out the lustre and smoothness desired.

The following example, which illustrates the preparation of a watch case or part of it, represents the preferred mode of carrying out the invention:

A mixture is prepared of 85 parts by volume of commercial grade tantalum carbide powder (which contains about 1% niobium carbide) and 15 parts of commercial nickel carbonyl powder. A sufficient amount of acetone is added to facilitate blending and the mixture is ground in a conventional ball mill having cemented carbide balls.

After the acetone evaporates and a fine homogeneous powder is obtained, the powder is wetted with a solution of camphor in ether. After, the ether evaporates, with the camphor remaining as a lubricant, the powder is poured into a mold and compressed at a pressure of 1500 kg. per cm.<sup>2</sup>. The pressed compacts are then pre-sintered for 15 minutes at 800° C. in a protective atmosphere formed by subjecting the sintering area to the action of a continuously acting vacuum pump. The pre-sintered compact is then machined with diamond tools and sintered again at 1450° C. for one hour under the same protective atmosphere. The sintered parts, after cooling, are then ground to the

required accurate dimensions and polished. The resulting products are used as watch casings and have the characteristic physical appearance of gold watch casings, but in addition, are considerably harder and more scratch resistant than the comparable gold products.

What is claimed is:

1. An article of jewelry having the color and physical appearance of gold and capable of being polished which consists essentially of a sintered mixture of between 70 and 90 parts by volume of at least one compound of the group consisting of tantalum carbide, zirconium nitride, titanium nitride and vanadium nitride and between 10 and 30 parts by volume of a metal of the group consisting of iron, cobalt, nickel and alloys thereof.
2. An article according to claim 1 in which said metal is of the group consisting of nickel and nickel base alloys.
3. An article according to claim 1 in which said metal is a nickel-chromium alloy containing about 5 to 50% by volume of chromium.
4. An article according to claim 1 containing zirconium nitride and a metal of the group consisting of nickel and nickel base alloys.
5. An article according to claim 1 containing titanium nitride and a metal of the group consisting of nickel and nickel base alloys.
6. An article according to claim 1 containing vanadium nitride and a metal of the group consisting of nickel and nickel base alloys.

7. An article according to claim 1 containing tantalum carbide and a metal of the group consisting of nickel and nickel base alloys.
8. An article according to claim 7 in which said metal is a nickel-chromium alloy containing about 5 to 50% by volume of chromium.

#### References Cited

#### UNITED STATES PATENTS

|           |         |              |          |
|-----------|---------|--------------|----------|
| 2,067,166 | 1/1937  | Balke        | 29—182.7 |
| 2,119,487 | 5/1938  | Padowicz     | 29—182.7 |
| 2,553,714 | 5/1951  | Lucas        | 29—182.7 |
| 2,979,811 | 4/1961  | Toney        | 29—182.7 |
| 3,165,822 | 1/1965  | Beeghly      | 29—182.7 |
| 3,369,892 | 2/1968  | Ellis et al. | 29—182.7 |
| 3,409,419 | 11/1968 | Yates        | 29—182.7 |
| 3,492,101 | 1/1970  | Prill et al. | 29—182.7 |
| 3,242,664 | 3/1966  | Lederrey     | 58—88    |

20 C. D. QUARFORTH, Primary Examiner

B. H. HUNT, Assistant Examiner

U.S. CL. X.R.

25 29—160.6, 182.5

UNITED STATES PATENT OFFICE  
CERTIFICATE OF CORRECTION

Patent No. 3,684,463

Dated August 15, 1972

Inventor(s) Franz Koelbl

It is certified that error appears in the above-identified patent and that said Letters Patent are hereby corrected as shown below:

In column 3 "90 parts" in line 10 should read -- 97% --; "and between 10 and" should be deleted in line 12; and "30 parts by volume of" in line 13 should read -- with the balance being --.

Signed and sealed this 3rd day of July 1973.

(SEAL)

Attest:

EDWARD M. FLETCHER, JR.  
Attesting Officer

Rene Tegtmeyer  
Acting Commissioner of Patents